

## UNITED STATES PATENT OFFICE.

ARLIE WILLIAM SCHORGER, OF MADISON, WISCONSIN, ASSIGNOR TO C. F. BURGESS  
LABORATORIES, OF MADISON, WISCONSIN, A CORPORATION OF WISCONSIN.

## METHOD FOR MAKING STEREOGRAPHIC MATS.

No Drawing.

Application filed November 30, 1923. Serial No. 677,880.

To all whom it may concern:

Be it known that I, ARLIE WILLIAM SCHORGER, a citizen of the United States, residing at Madison, in the county of Dane, 5 State of Wisconsin, have invented certain new and useful Improvements in Methods for Making Stereotype Mats; and I do hereby declare the following to be a full, clear, and exact description of the invention, such 10 as will enable other skilled in the art to which it appertains to make and use the same.

The rapidity with which modern newspapers are printed is due largely to use of the 15 stereotype mat, also known as a "matrix", or "flong". As soon as a form containing the type has been set up, a stereotype mat is superimposed, then covered with blankets or felts and passed through a rolling machine, whereby the mat requires a reverse impression of the type. The mat after drying is placed in a casting machine where it is held in the form of a cylinder. Molten stereotype metal is now poured into the machine whereby a metal cylinder is obtained containing on its surface an exact duplicate of the type in the original flat form.

The cylindrical stereotype plate is then placed in a cylinder press whereby papers 30 can be printed at high speed. Several casts can be made easily and rapidly from the same mat so that a number of presses can be placed in operation almost simultaneously.

There are two types of stereotype mats in 35 commercial use, the so-called "wet mat" and the "dry mat". The "wet mat", which is in most extensive use, consists of two or three sheets of thin blotting paper and two to four sheets of tissue paper held together by a paste made of starch, dextrin, gum arabic, etc. The tissue is used on the face to obtain a sharp, smooth impression. The wet mat, after having been built up, must 40 be stored in a wet condition. This is a serious objection. Furthermore, it must be dried on the type form as otherwise it would warp and shrink greatly. Considerable labor and much skill, judgment and experience is required to produce a satisfactory 45 wet mat. The rush of work in a newspaper press room cannot tolerate unreliability in the quality of the mats supplied to the casting machine. Without suitable mats the printing cylinders cannot be made and with- 50

out these the printing can not proceed. In a modern newspaper office an interruption or even delay incident to bad workmanship on the wet mats, or unreliability in the starch with which they are made is a serious 55 matter. They have to be made up shortly prior to the time fixed for their use and without adequate opportunity for testing, excepting by actual use. But by the time defects in material and workmanship develop, the harm has been done to the printer and to all those ramifications of the newspaper art which are dependent on the timely issuance of the paper from the press.

The "dry mat" on the other hand, can be 60 stored in the dry state in any quantity, but previous to use must be "conditioned" by being placed in a humidor where it takes up from 10 to 30% of moisture. It is then rolled on the form, removed, placed in a 65 cylindrical "scorcher" where most of the moisture is removed in one or two minutes. It is then ready for use in the casting machine. From the standpoint of initial cost, speed, and ease of manipulation it is preferable to use a dry mat instead of a wet mat. In getting out a "rush" edition where every 70 second counts, it is obvious that greater speed can be obtained with a dry mat.

The objection to the dry mat as now being manufactured is that it has a rougher surface than the wet mat and does not give satisfactory impressions with half-tone blocks with a fine screen, and in general, lacks sharpness of definition. The dry mat 75 does not have the plasticity of a wet mat, so that fractures may be produced during molding on the type, into which the molten stereotype metal will run. On removing the casting, the face of the mat will be torn 80 so that the mat cannot be used for a second casting. A properly made mat should permit the making of 10 to 20 casts. The fractures and roughness characteristic of the present dry mat is largely due to the character of the fibers employed. If they are long and the surface roughens readily so that loose fibers are produced, the molten metal will flow amid the fibers, the surface of the mat becoming torn when the casting is removed, so that both the casting and the mat 85 may be rendered useless.

It is not possible to obtain a satisfactory mat by the use of large quantities of adhesives, such as are frequently employed, 90 ow- 95

100 105 110

ing to the fact that the mat when dry is not plastic, and if used wet it has all the disadvantages already pointed out.

With my invention, as will be described below, these objections are overcome by the use of relatively fine, short, soft fibers, formed into a sheet to give an article having a high degree of smoothness, strength and impressionability.

- 10 The natural cellulosic fibers available for manufacture of paper are so long and smooth that when a sheet formed from them is subjected to a strain, the fibers either slip past one another or are ruptured. In either case a roughness is produced that permits the metal to run into the mat. This difficulty cannot be overcome by simply shortening the fibers by cutting, since, in this case the sheet would have very little strength. In my process these objections are overcome by cutting and splitting the fibers into fine fibrils. Rag stock, cotton linters, wood pulp and similar fibers, either alone or mixed, are placed in a paper-maker's beater, or other suitable apparatus and while suspended in water are subjected to a cutting and splitting action by suitably adjusting the beater roll with respect to the bed plate. After sufficient beating, the original fibers will have been shortened in length and split longitudinally into small fibrils. The splitting action is complete in some fibers; in others the ends are separated into brushes and the fibrils formed on the sides of the fiber give an arborescent appearance. The difference between the fibers before and after beating cannot well be shown in a pen and ink drawing, but is readily apparent under a microscope, particularly, if the fibers are stained in well known manner. The relatively prolonged beating in water separates the fibers from one another by combing out the pulp and without undue cutting or breakage of the whole fibers develops the fibrillated condition so important to the successful practice of the present invention. When the fibers are combed out as described above and made into a sheet on the paper machine, the individual fibers are so interlocked by reason of the fibrils that stick out along the sides and ends of the individual fibers that the sheet as a whole acts somewhat like a net permitting the required amount of stretching and plasticity during molding against the type, but with adequate strength to permit the sheet subsequently to be rolled into cylindrical form and with all the toughness and heat resistance needed for a subsequent repeated contact with hot metal.

In beating the fibers to the necessary state of fibrillation they unavoidably become hydrated or gelatinized on the surface, some of the smaller fibers, or fibrils formed from them, may be completely converted to

a structureless mass of gelatinized cellulose. Gelatinized cellulose per se has the characteristic that when dried it hardens to a horn like mass, dark gray in color, and very hard and brittle. During the change to the hard horny mass the shrinkage of the material is enormous, and there is a pronounced tendency to warp and curl.

In beating the fibers, as above described, gelatinization occurs to such an extent that if the stock were made into a sheet and allowed to dry, the sheet would become hard and brittle and have a low receptivity to impression. I have found that by heating the pulp in an alkaline solution the gelatinized cellulose is destroyed, or removed, leaving behind clean ungelatinized fibrillated fibers of excellent felting properties and with no tendency to become hard or brittle on drying. The heating or cooking may be performed at atmospheric pressure or at a steam pressure of 5 to 20 pounds. The amount of chemical used and the cooking conditions employed will vary with the nature of the pulp, and the degree of beating. But with an easy-bleaching sulphite wood pulp, after fibrillation as described above, the alkaline cooking solution may properly contain 10% of caustic soda based on the weight of the pulp, and the cooking may be continued until the liquor is no longer alkaline to litmus. The resulting fibers, after washing with water, are unchanged in form, but are lighter in color, soften on drying and possessed of a high degree of plasticity when in sheet form. It will be understood, of course, that other alkalis and alkaline earths may also be employed in the cooking liquor.

The fibers, fibrillated and cooked as described above are thoroughly washed, mixed with a paper maker's clay, and made into mats of the desired thickness, usually about 0.030 inch. It is preferable to build up a mat in several layers as this procedure gives greater uniformity and strength. Eight to ten layers have been found very satisfactory. This can be done by the use of various types of paper machines known to those skilled in the art.

The clay impregnates the entire sheet by filling in the small interstices between the fibers, and the finished mat is strong, flexible and free from crevices. It may be dried and stored like ordinary paper stock, and the quality of any batch may be tested out long in advance of the time for using the batch in commercial press room work.

To put the sheets or mats in condition for any use it is only necessary to bring up their moisture content in a humidor to that content best suited to the needs of the moment. A moisture content of 10 to 30% before "scorching" will be found suitable for most work.

A stereotype mat made as above described

even though classifiable as a dry mat and not a wet mat will give clear, deep and sharp impressions having smooth dense surfaces. It may be used for fine line reproductions with much the same results as from the use of a wet mat and without any of the worrying uncertainties incident to wet mat production.

I claim:

- 10 1. A stereotype mat composed essentially of fibrillated fibers and a filler; substantially as described.
- 15 2. A stereotype mat composed essentially of fibrillated cellulose fibers and a mineral filler.
- 20 3. A stereotype mat composed of a plurality of superposed layers of fibrillated cellulose fibers, and a filler.
- 25 4. A stereotype mat comprising clean un-gelatinized fibrillated fibers impregnated with clay.
- 30 5. A stereotype mat consisting essentially of clay and fibrillated cellulose fibers freed from gelatinized cellulose by cooking with alkali; substantially as described.
- 35 6. A stereotype mat comprising a plurality of superposed layers felted together, each of said layers consisting essentially of clay and of cellulose fibers that have been

fibrillated by beating in water and purified 30 of gelatinized cellulose by heating in alkali, substantially as described.

7. The method of making a dry mat which consists in beating cellulosic material until the fibers develop fibrils, cooking in alkali 35 to remove gelatinized cellulose, mixing with a filler and forming into sheets; substantially as described.

8. As a step in the manufacture of stereotype dry mats, the process which consists 40 in beating cellulosic material until the fibers are split, in part at least, into fibrils, and then cooking in alkali to remove gelatinized cellulose and soften the fibrillated fibers.

45 9. The method of making a dry mat which consists in beating cooked wood pulp in water until the fibers separate and develop fibrils, cooking the fibrillated fibers in alkali to free the fibers from gelatinous material, 50 washing in water, mixing with clay, forming into sheets composed of a plurality of like layers felted together and allowing said sheet to dry; substantially as described.

55 In testimony whereof I affix my signature.

ARLIE WILLIAM SCHORGER.